

April 28, 1936.

K. HAYAKAWA

2,039,165

## METHOD OF TREATING ALUMINIUM OR ALUMINIUM ALLOY

Filed Jan. 17, 1935

Fig. 1.



Fig. 3.



Fig. 2.



INVENTOR.  
KAZUMA HAYAKAWA  
BY *Haseltine, Lake & Co.*  
ATTORNEYS.

## UNITED STATES PATENT OFFICE

2,039,165

METHOD OF TREATING ALUMINIUM OR  
ALUMINIUM ALLOYKazuma Hayakawa, Hodogaya-ku,  
Yokohama, Japan

Application January 17, 1935, Serial No. 2,171

2 Claims. (Cl. 75—68)

The present invention relates to a method of treating aluminium or aluminium alloy which is based on the knowledge that when the gas contained in aluminium or aluminium alloy is liberated by heating them in vacuum, it reacts with aluminium and iron and produces various compounds having high hardness and that said compounds are turned into fine particles by ageing and distributed all over the aluminium or aluminium alloy, thus producing aluminium or aluminium alloy having high hardness as a whole, characterized by the fact that molten aluminium or aluminium alloy is put into an iron vessel and heated in vacuum for thirty to sixty minutes at a temperature above 900° C., after which the heating temperature is lowered to 500° to 700° C. and hydrocarbon gas is filled in the vessel up to more than 1 atm. and then the material is cooled rapidly.

20 The object of this invention is to obtain aluminium or aluminium alloy having high hardness simply by considerably increasing the hardness of aluminium or aluminium alloy easily and effectively.

25 Generally, aluminium solution possesses the property of absorbing a gas very much, so it is made to be able to absorb in a molten state a gas having the volume

30  $\frac{1}{10}$  to  $\frac{1}{13}$

and at the higher temperature it can absorb the bigger quantity. According to Gwyer (Trans. Faraday Soc. 1919, vol. 14, p. 173), the following gases were absorbed:—

|                 | Percent   |
|-----------------|-----------|
| Carbon dioxide  | 3 - 8     |
| Carbon monoxide | 0 - 9.5   |
| 40 Hydrogen     | 55 - 81   |
| Methane         | 1 - 24.5  |
| Nitrogen        | 5 - 11    |
| Oxygen          | 1.5 - 4.5 |

45 Of them, those which act upon aluminium at a high temperature are carbon monoxide and carbon dioxide and make the following chemical changes:



When the free carbon thus produced comes into contact with aluminium in vacuum, it will produce crystals of  $\text{Al}_4\text{C}_3$  at 650° C. On the other hand, aluminium has iron melted thereinto at a

high temperature in the presence of hydrogen and produces  $\text{FeAl}_3$ . Consequently, hard compounds, namely,  $-\text{FeAl}_3$ ,  $\text{Al}_4\text{C}_3$  and  $\text{Al}_2\text{O}_3$  are distributed in aluminium or aluminium alloy at a high temperature and are present therein in a saturated condition. However, if cooled rapidly, they take an oversaturated condition at the ordinary temperature and then, with the lapse of time, are turned into a fine state and separated from the solid solution. Thus, it is possible to obtain aluminium or aluminium alloy having high hardness.

Referring to the appended drawing,

Fig. 1 is a longitudinal elevation of an apparatus employed for carrying out this invention into practice;

Fig. 2, a section cut off along the line II—II of Fig. 1 and

Fig. 3, a section showing the condition in which fine crystals of  $\text{FeAl}_3$ ,  $\text{Al}_4\text{C}_3$  and  $\text{Al}_2\text{O}_3$  have been distributed in aluminium metal and hardened very high.

To explain the present method with reference to the accompanying drawing,

In Figure 1, 1 is an ingot of aluminium or aluminium alloy; 2, an iron vessel, for example, an iron pot; 3, an electric resistance furnace and 4, the part where two flat surfaces are connected together by friction, 6 is a porcelain tube for supporting the lead wire 7 of said electric resistance furnace 3, said lead wire 7 being cemented to said tube 6 at its end with Dekotinsky cement. 8 is a water jacket; and 9, an empty chamber to be rendered vacuous or cooled as necessary. If air is exhausted from tubes 14 and 15, closing cocks 10, 11 and 12 and opening a cock 13 and operating an air pump (not shown), the above empty chamber 9 will be rendered vacuous. Reversely, if water is introduced into said chamber 9 from a conduit 16, closing the cock 13 and opening the cocks 10 and 11, and then the filling water is discharged from an exhaust pipe 17 through the cock 18, it is possible to cool the chamber. 18 is a heat resisting steel plate adapted for preventing the deformation of the furnace wall by reflecting heat. 19 is a heat reflecting plate consisting of a round heat resisting steel plate having apertures 20 and a heat resisting steel plate of the smaller diameter, combined to form an I-shaped section. It is engaged with the projections 21 of the upper part of the inner wall of the furnace and is suspended over the iron pot 2. The exhaust of the air in the furnace is effected from a tube 15 through the apertures 20 of the heat reflecting plate 19 by means of an air pump (not shown).

Also, to fill hydrocarbon gas in the furnace, it is introduced into the latter from the tube 15 through a tube 22 and the cock 12.

The following is the manner of performing this invention by employing the above apparatus:—

Firstly, closing the cocks 10, 11 and 12 and opening the cock 13, exhaust air from both the furnace and empty chamber 9 by an air pump till they become partially vacuous, when the interior 10 of the furnace is heated by the electric resistance furnace 3, and as the empty chamber 9 is at this time in a vacuous state, it prevents the escape of heat from the electric furnace 3. Thus, after melting aluminium or aluminium alloy by 15 heating it in the iron pot 2 for thirty to sixty minutes by said electric furnace, lower the temperature to 500-700° C. by regulating the voltage of the electric furnace. Then, fill hydrocarbon gas in the furnace up to over 1 atm. through the tube 15 from the tube 22 by opening the cock 12. Soon after, opening the cocks 10 and 11 and closing the cocks 12 and 13, introduce cooling water into the empty chamber 9 from the tube 16 and discharge it from the tube 17, thus cooling said 25 molten aluminium or aluminium alloy rapidly.

The aluminium or aluminium alloy thus obtained having fine crystals of  $FeAl_3$ ,  $Al_4C_3$  and

$Al_2O_3$  distributed all over them as shown in Figure 3, possesses very high hardness.

In Figure 3, 23 is the outer cylindrical part of an iron vessel having the hardness 10.2° according to Rockwell scale. 24 is the aluminium metal 5 manufactured according to the present invention, the hardness of the different parts of which, when measured with Rockwell scale, has the values as shown in Fig. 3.

I claim:

1. Method of treating aluminium or aluminium alloy, which consists in heating molten aluminium or aluminium alloy in vacuum in an iron vessel for thirty to sixty minutes at over 900° C., then lowering the heating temperature to 500 to 700° 15 C. and filling hydrocarbon gas in said vessel up to over 1 atm. and subsequently cooling the above material quickly.

2. Aluminium or aluminium alloy having high hardness, which is made by heating molten aluminium or aluminium alloy in vacuum in an iron vessel for thirty to sixty minutes at over 900° C., then lowering the heating temperature to 500 to 700° C. and filling hydrocarbon gas in said vessel up to over 1 atm. and subsequently cooling the 25 above material quickly.

KAZUMA HAYAKAWA.